# EUROPEAN PATENT SPECIFICATION

(11) **EP 1 216 759 B1**
(45) Date of publication and mention of the grant of the patent: **01.02.2012**
(21) Application number: 01130594.3
(22) Date of filing: 21.12.2001
(51) Int. Cl.: B05D 1/28, B05D 3/02

(54) **Method and unit for producing highly abrasion-resistant protective coverings, in particular for floor and work surfaces**
Verfahren und Anlage zur Herstellung von einer hochabriebfesten Beschichtung insbesondere für Bodenbeläge und Werkstückoberflächen
Procédé et installation pour produire un revêtement hautement résistant à l'abrasion en particulier pour les sols et les surfaces de travail

(30) Priority: 22.12.2000 IT MI002813
(43) Date of publication of application: 26.06.2002
(73) Proprietor: Tocchio S.r.l., 27029 Vigevano (IT)
(72) Inventor: Tocchio, Umberto, 27029 Vigevano (IT)
(74) Representative: Cerbaro, Elena

(56) References cited:
- EP-A1- 0 511 129
- WO-A-02/43879
- DE-C- 19 814 212
- US-A- 4 675 208
- US-A- 4 968 538
- US-A- 5 306 523
- US-E- R E30 691

## Description

The present invention relates to a method for producing highly abrasion-resistant protective coverings, particularly for floor and work surfaces, but which may also be used for other applications (e.g. walls or furniture).

As is known, laminated panels are widely used for covering floors, as an alternative to conventional woodblock floors, or for covering walls, furniture, etc., and normally comprise a number of layers of sheet material (e.g. paper or fabric) impregnated with thermosetting polymer resin (e.g. phenolic, urea, melamine resins or mixtures of these) and which are gripped and compressed under heat (consequent polymerization/cross-linking of the resin compacts the layers to form the panel).

The eventually visible layer is normally patterned to reproduce a given design (e.g. a given wood grain), and the patterned layer is covered with a protective abrasion-resistant covering or so-called "overlay" containing powdered aluminium oxide Al₂O₃ (corundum) or other abrasion-resistant substances.

More specifically, as a protective covering, an overlay paper is known to be used, in which corundum particles are incorporated directly, and which is then impregnated with resin, applied on the patterned layer, and hot-pressed. The method of producing powdered corundum paper is extremely expensive and complicated, and fails to ensure uniform particle distribution (essential for good abrasion resistance).

Alternatively, abrasion-resistant powder is applied to a wet preimpregnated substrate (i.e. impregnated with resin not yet dried or cross-linked) prior to the final pressing. More specifically, in EP-A-329154, pure abrasion-resistant powder is applied directly to the wet preimpregnated substrate; whereas, in DE-A-19814212, abrasion-resistant powder is dispersed in a resin, and the mixture sprayed on to the wet preimpregnated substrate. In both cases, the abrasion-resistant powder is applied to a wet preimpregnated substrate, and neither completely solves the problem of uniform dispersion of the abrasion-resistant powder, so that the resulting laminates are not always satisfactory in terms of abrasion resistance.

It is an object of the present invention to provide a method of producing highly abrasion-resistant protective coverings, in particular for floor and work surfaces, designed to eliminate the aforementioned drawbacks of known methods, and which at the same time is relatively cheap and easy to implement, and provides for obtaining products with an abrasion resistance superior to that obtained using known methods.

According to the present invention, there is provided a method for producing highly abrasion-resistant protecting coverings, in particular for floor and work surfaces, as claimed in claim 1.

Here and hereinafter:
- "thermosetting polymer resin" is intended to mean a polymer system of one or more components, which sets irreversibly by polymerization and/or cross-linking reactions; as is known, depending on the polymer components used, the setting process can be activated, for example, by heat and/or electromagnetic radiation and/or with the aid of catalysts;
- "sheet material" is intended to mean a thin material in the form of a continuous strip or single sheet (e.g. paper, fabric, etc);
- "powdered abrasion-resistant substance" is intended to mean a solid substance in the form of particles (microspheres, granules, crystals, and particles of any sort) and of superior hardness and abrasion resistance (e.g. metal oxides, silicates or ceramics).

Preferably, the thermosetting polymer resins employed according to the present invention are water-base resins selected, for example, from the group comprising melamine, phenolic, urea resins and mixtures of these; and the powdered abrasion-resistant substance is aluminium oxide (Al₂O₃, corundum).

It is important that, before the resin and abrasion-resistant substance mixture is applied, the sheet material has a relatively low wet residue of volatile substances, in particular, below approximately 14% by weight (determined in an oven at 160° for 5 minutes).

The sheet material may be nonimpregnated paper material or preimpregnated so-called "prepreg" sheet material; in which latter case, the method comprises the steps of: i) impregnating said sheet material with a second thermosetting polymer resin; ii) drying said preimpregnated sheet material to cross-link said second thermosetting polymer resin; and, iii) applying and distributing said mixture evenly on at least one surface of the dried said preimpregnated sheet material.

In this case, too, it is important that, after drying and before applying the resin and abrasion-resistant substance mixture, the dried preimpregnated sheet material has a low wet residue of volatile substances, in particular, of 7 to 14% by weight (determined in an oven at 160° for 5 minutes).

The thermosetting polymer resin mixed with the abrasion-resistant substance is continuously agitated and kept in preferably turbulent motion, both when preparing the mixture and when applying the mixture to the sheet material, to prevent the powdered abrasion-resistant substance (which has a higher density than the resin in which it is dispersed) from settling, and to ensure it is evenly distributed in the resin when applied to the sheet material. Turbulent motion of the mixture has proved particularly advantageous.

In a preferred embodiment, the step of applying the resin and abrasion-resistant substance mixture is performed using a dispenser-applicator device comprising a fountain, and at least one applicator roller positioned substantially contacting said first surface of the sheet material along a generating line of contact to transfer said mixture from said fountain to said first surface, whereas, on a second surface, opposite said first surface, of the sheet material and at said generating line of contact, no support for said sheet material is provided.

The method also comprises a step of recirculating the resin and abrasion-resistant substance mixture, in which said mixture dispensed by said fountain and not deposited on said first surface of the sheet material is recirculated back to said fountain.

When preparing the resin and abrasion-resistant substance mixture, at least one viscosity-control additive, selected from the group comprising filmogens and preferably capable of thermal three-dimensional cross-linking, may be added to the mixture. Good results have been obtained, for example, using a viscosity regulator of polyvinyl alcohol (PVA), which also keeps the volatile substances in the mixture low (below approximately 5% by weight) and so prevents powder dispersion in the workplace. Once dehydrated, PVA also leaves a film which does not affect the original colour of the paper (or other substrate) on which it is applied.

An important aspect of the invention is that said step of applying the resin and abrasion-resistant substance mixture and said step of drying the sheet material coated with the mixture are followed by a further step of applying a layer of a third thermosetting polymer resin, which is in turn dried and/or polymerized-cross-linked. This third resin, hereinafter referred to as "protective resin", is also preferably a water-base resin selected, for example, from the group comprising melamine, phenolic, urea resins and mixtures of these. The protective resin may be applied 100% dry or in a wet phase, and may or may not contain various additives, cross-linking-polymerization catalysts, etc. Most preferably, a particle filler (in the form of microspheres, granules, powder, crystals, etc.) of nonabrasive or relatively nonabrasive solid substances (e.g. metal oxides, silicates or ceramics) is dispersed in the protective resin. The function of the protective-resin layer is to prevent wear of the plates (normally chromium-plated) used to hot-press the covering. Applying the protective resin, preferably with a particle filler, prevents the plates from coming into direct contact with the very hard abrasion-resistant substance in the underlying layer, and so protects the plates against relatively rapid wear.

The protective resin (possibly with a dispersed particle filler) may also be applied using a dispenser-applicator device identical to that used to apply the first thermosetting polymer resin and powdered abrasion-resistant substance mixture.

The step of applying the resin and abrasion-resistant substance mixture and the step of drying the sheet material coated with the mixture may be performed repeatedly to form respective superimposed cover layers. Likewise, the step of applying the protective resin (with or without the filler) may also be repeated to form respective superimposed layers.

Both the step of drying the sheet material coated with the resin and abrasion-resistant substance mixture and the step of drying the protective resin may be conducted to only dry the polymer components by more or less drastic removal of the volatile substances, or to produce a complete or only partial polymerization-cross-linking reaction of the polymer components. Depending also on the type of polymer components used, the drying steps may be conducted in a tunnel furnace, or by infrared or ultraviolet lamp or electron beam radiation.

After the drying step/s, the sheet material coated with the resin and abrasion-resistant substance mixture (and possibly also the protective resin) is ready for use, e.g. for the next (known) hot-pressing step in which the polymerization-cross-linking reaction of the polymer resins may be completed.

Buffered acid catalysts are preferably added to the resin and abrasion-resistant substance mixture to control the cross-linking reaction. More specifically, the catalysts are such as to bring about the cross-linking reaction, in 100°C boiling water conditions, in about 200 seconds, and at any rate in less than 4 minutes. The sheet material impregnated with the resin and abrasion-resistant substance mixture (and possibly with the protective-resin layer) is pressed to achieve a high degree of cross-linking (the viscosity-control additive is advantageously also a three-dimensional cross-linking agent for enhancing cross-linking, such as PVA).

The method according to the invention is easy and relatively cheap to implement; the unit implementing it is cheap and easy to produce and operate; and coverings produced using the method and unit according to the invention have proved more resistant to abrasion than similar coverings or panels produced using known methods, as confirmed by comparative tests. More specifically, abrasion tests were conducted (in accordance with proposed European standard pr-EN-13329, not yet in force but already adopted in the industry as a reference standard) of coverings produced according to the invention, and similar coverings produced using conventional methods : the coverings produced according to the invention were classed AC3 (suitable for heavy-duty flooring), as compared with class AC2 for conventional coverings. The method according to the invention is therefore not only easier to implement and more effective than known methods, but also provides for obtaining better results.

Purely by way of example, excellent results have been obtained using a mixture of melamine resin (supplier: BASF) with a 60% solid content, and powdered corundum (supplier: Baikowsky): the mixture, with a 25-second viscosity in a Ford 4 cup at 20°C and a 65% solid content, was spread on to the sheet material in an amount corresponding to 40 g/m² of resin and 16 g/m² of corundum.

A number of non-limiting embodiments of the present invention will be described by way of example with reference to the accompanying drawings, in which:
Figure 1 shows a schematic side view of a unit for producing protective coverings for laminated panels and implementing the method according to the invention;
Figures 2 and 3 show schematic, larger-scale views of variations of a detail of the Figure 1 unit.

Number 1 in Figure 1 indicates as a whole a unit for producing highly abrasion-resistant protective coverings, in particular for floor and work surfaces.

Unit 1 comprises preparing means 2 for preparing a mixture 3 containing a powdered abrasion-resistant substance 4 dispersed evenly in a liquid thermosetting polymer resin 5; feed means 6 for feeding a sheet material 7; a dispenser-applicator device 8 for applying mixture 3 on to a first surface 9 of sheet material 7; and drying means 10 downstream from dispenser-applicator device 8.

In the non-limiting example shown, preparing means 2 comprise two tanks 11, 12 arranged in series and having respective agitators 13, 14; and a feeder 15 (e.g. a screw) for feeding abrasion-resistant substance 4 into tank 11. Tank 12 is connected to dispenser-applicator device 8 by a feed line 16 fitted with a circulating pump 17; a recirculating line 18 feeds part of the mixture 3 drawn from tank 12 back into tank 12; and circulating pump 17 keeps mixture 3 in constant, preferably turbulent, motion between tank 12 and dispenser-applicator device 8. Means 6 for feeding sheet material 7 are known and therefore not described or illustrated in detail for the sake of simplicity. Though reference is made in the present disclosure to a sheet material 7 in the form of a continuously treated strip, it is understood that unit 1 may process individual sheets of sheet material 7. Dispenser-applicator device 8 comprises a fountain 19; and at least one applicator roller 20 positioned substantially contacting first surface 9 of sheet material 7 along a generating line of contact. Supporting means 21, 22 for supporting sheet material 7 and defined, in the example shown, by respective rollers are provided on opposite sides of applicator roller 20 to keep the sheet material suspended; and, at the generating line of contact of applicator roller 20, a second surface 23, opposite first surface 9, of sheet material 7 has no support, so that sheet material 7 simply spans rollers 21 and 22.

Dispenser-applicator device 8 also comprises agitating means 24 defined, for example, by a powered arm 25 moving inside fountain 19 to continuously agitate and keep the mixture 3 inside fountain 19 in preferably turbulent motion.

Unit 1 also comprises recirculating means 26 for recirculating mixture 3 from dispenser-applicator device 8 to tank 12, and which comprise a catch tank 27 located beneath dispenser-applicator device 8 and facing second surface 23 of sheet material 7, and a recirculating line 28 connecting catch tank 27 to tank 12 and fitted with a recirculating pump 29. Unit 1 may also comprise finish rollers 30 of any known type downstream from dispenser-applicator device 8 and upstream from drying means 10.

Figures 2 and 3 show various detailed embodiments of dispenser-applicator device 8. In the Figure 2a embodiment (corresponding to the one in Figure 1), dispenser-applicator device 8 comprises applicator roller 20 and a dispensing roller 31 : applicator roller 20 and dispensing roller 31 are positioned side by side along respective generating lines, are separated by an axial gap through which mixture 3 flows, and together define fountain 19; the mixture 3 from preparing means 2 is fed between applicator roller 20 and dispensing roller 31; applicator roller 20 transferring mixture 3 from fountain 19 to sheet material 7 is positioned contacting surface 9 (the top surface) of sheet material 7; and dispensing roller 31 is detached from sheet material 7. Preferably (though not necessarily), the rotation direction of applicator roller 20 is such that, at the point at which the mixture is applied, applicator roller 20 moves in the opposite direction to sheet material 7. As opposed to being located over sheet material 7 (as in Figure 2a), dispenser-applicator device 8 may obviously be located beneath sheet material 7, as shown in the Figure 2b variation (in which case, surface 9 of the sheet material to which mixture 3 is applied is the bottom surface). Dispensing roller 31 may rotate in the opposite direction to applicator roller 20 (as shown by the continuous arrows in Figures 2a and 2b) or in the same direction (as shown by the dash arrows).

In the Figure 2c and 2d variations, dispenser-applicator device 8 comprises an applicator roller 20; and two dispensing rollers 31, 32 detached from sheet material 7 and positioned facing each other a small distance apart to define fountain 19. Applicator roller 20 is positioned contacting sheet material 7 and facing dispensing roller 31. Dispensing rollers 31, 32 may, obviously, be positioned otherwise than as shown with respect to applicator roller 20 and sheet material 7. For example, in Figure 2d, dispensing rollers 31, 32 are aligned in a direction substantially parallel to sheet material 7. Dispensing rollers 31, 32 may be rotated in opposite directions (as shown by the continuous arrows in Figures 2c and 2d) or in the same direction (as shown by the dash arrows).

In the Figure 2e, 2f variations, dispenser-applicator device 8 comprises an applicator roller 20 contacting sheet material 7; and a doctor 33 cooperating in sliding manner with applicator roller 20. In this case, fountain 19 is defined between applicator roller 20 and doctor 33, and the mixture 3 from preparing means 2 is fed between applicator roller 20 and doctor 33.

As stated, the rotation direction of applicator roller 20 may be such that, at the point at which mixture 3 is applied to sheet material 7, applicator roller 20 moves in the opposite direction to sheet material 7 (as shown in Figure 2). Alternatively, the rotation direction of applicator roller 20 may be such that, at the point at which mixture 3 is applied to sheet material 7, applicator roller 20 moves in the same direction as sheet material 7, as shown in Figure 3 (which shows the same embodiments of dispenser-applicator device 8 as in Figure 2, but with applicator roller 20 rotating in the opposite direction).

Operation of unit 1 implementing the method according to the invention described above is as follows.

Abrasion-resistant substance 4 and resin 5 are fed into and mixed and agitated continuously in tank 11 (possibly together with the additives and catalysts mentioned previously); when abrasion-resistant substance 4 is evenly dispersed in resin 5, mixture 3 is drained into tank 12, mixed further, and fed along feed line 16 to fountain 19; and, in the meantime, dry sheet material 7 (which may be a strip of paper or other nonimpregnated material or a dried preimpregnated material) is supplied.

By means of dispenser-applicator device 8, mixture 3 is applied and spread evenly on surface 9 of sheet material 7; sheet material 7 spread with mixture 3 is then fed to drying means 10 (e.g. an oven) from which emerges a covering 35 comprising a substrate defined by sheet material 7, and a layer of resin 5 incorporating powdered abrasion-resistant substance 4.

Circulating pump 17, recirculating pump. 29, and agitators 13, 14 continuously agitate and keep mixture 3 in preferably turbulent motion to prevent abrasion-resistant substance 4 (which has a higher density than resin 5) from settling.

Mixture 3 is applied by dispenser-applicator device 8 by means of applicator roller 20, which transfers mixture 3 from fountain 19 to sheet material 7. Any mixture 3 not deposited on sheet material 7 (e.g. dripping from the axial ends of applicator roller 20) is collected in tank 27 and recirculated. Not providing any support for sheet material 7 on the surface 23 side opposite surface 9 prevents mixture 3 from depositing on and impairing operation of a contrast roller or other mechanical member.

The amount of mixture 3 dispensed by dispenser-applicator device 8 and applied to sheet material 7 may be controlled effectively by regulating the rotation speed of applicator roller 20 and/or dispensing rollers 31, 32.

Clearly, changes may be made to the method and unit as described and illustrated herein without, however, departing from the scope of the present invention.

## Claims

1. A method of producing highly abrasion-resistant protective coverings, in particular for floor and work surfaces, comprising the steps of:
a) preparing a mixture of a powdered abrasion-resistant substance dispersed evenly in a first thermosetting polymer resin;
b) providing a substantially dry sheet material having a low wet residue of volatile substances;
c) applying and distributing said mixture evenly on at least one surface of said substantially dry sheet material;
d) drying said sheet material coated with said mixture to form a covering incorporating said powdered abrasion-resistant substance;
the method being **characterized by** also comprising, after said step of applying said mixture and said step of drying said sheet material coated with said mixture, the steps of:
e) applying to said covering incorporating said powdered abrasive-resistant substance at least one layer of a third thermosetting polymer resin having a particle filler of nonabrasive or relatively nonabrasive solid substances dispersed therein; and
f) drying said third resin.

2. A method as claimed in Claim 1, **characterized in that**, prior to applying said mixture, said substantially dry sheet material has a wet residue of volatile substances (determined in an oven at 160° for 5 minutes) of less than approximately 14% by weight.

3. A method as claimed in Claim 1 or 2, **characterized in that** said sheet material is a nonimpregnated paper material.

4. A method as claimed in Claim 1 or 2, **characterized in that** said sheet material is a preimpregnated, so-called "prepreg" sheet material; in which case, the method comprising the steps of : i) impregnating said sheet material with a second thermosetting polymer resin; ii) drying said preimpregnated sheet material to polymerize-cross-link said second thermosetting polymer resin; and, iii) applying and distributing said mixture evenly on at least one surface of the dried said preimpregnated sheet material.

5. A method as claimed in Claim 4, **characterized in that**, after drying and before applying said mixture, said dried preimpregnated sheet material has a wet residue of volatile substances (determined in an oven at 160° for 5 minutes) of 7 to 14% by weight.

6. A method as claimed in one of the foregoing Claims, **characterized in that** said first thermosetting polymer resin is continuously agitated and kept in preferably turbulent motion during said steps of preparing and applying said mixture.

7. A method as claimed in one of the foregoing Claims, **characterized in that** said step of applying said mixture is performed by a dispensing device comprising a fountain, and at least one applicator roller positioned substantially contacting said first surface of the sheet material along a generating line of contact to transfer said mixture from said fountain to said first surface; whereas, on a second surface, opposite said first surface, of the sheet material and at said generating line of contact, no support for said sheet material is provided.

8. A method as claimed in the foregoing Claim, **characterized by** also comprising a step of recirculating said mixture, and in which said mixture dispensed by said fountain and not deposited on said first surface of the sheet material is salvaged and fed back to said fountain.

9. A method as claimed in one of the foregoing Claims, **characterized in that**, during said step of preparing said mixture, at least one viscosity-control additive, selected from the group comprising filmogens and preferably capable of thermal three-dimensional cross-linking, is added to said mixture.

10. A method as claimed in one of the foregoing Claims, **characterized in that** said thermosetting polymer resins are water-base resins selected, for example, from the group comprising melamine, phenolic, urea resins and mixtures thereof; said powdered abrasion-resistant substance being aluminium oxide (Al₂O₃, corundum).

11. A method as claimed in one of the foregoing Claims, **characterized in that** said steps of applying said mixture and drying said sheet material coated with said mixture are repeated one or more times to form respective superimposed cover layers.

## Patentansprüche

1. Verfahren zum Herstellen von hoch abriebfesten Schutzbelägen, insbesondere für Boden- und Arbeitsflächen, umfassend die Schritte:
a) Erzeugen einer Mischung einer pulverförmigen abriebfesten Substanz, die gleichmäßig in einem ersten Duroplastharz dispergiert ist;
b) Bereitstellen eines im Wesentlichen trockenen bahnenförmigen Materials mit einem niedrigen Nassrückstand an flüchtigen Substanzen,
c) gleichmäßiges Auftragen und Verteilen der Mischung auf wenigstens einer Oberfläche des im Wesentlichen trockenen bahnenförmigen Materials
d) Trocknen des bahnförmigen Materials, das mit der Mischung beschichtet ist, um einen Belag zu bilden, der die pulverförmige abriebfeste Substanz umfasst;
wobei das Verfahren **dadurch gekennzeichnet ist, dass** es nach dem Schritt des Auftragens der Mischung und dem Schritts des Trocknens des bahnenförmigen Materials, das mit der Mischung beschichtet ist, auch folgende Schritte umfasst:
e) Auftragen auf den Belag, der die pulverförmige abriebfeste Substanz umfasst, wenigstens einer Schicht eines dritten Duroplastharzes worin ein Partikelfüller aus nicht abriebfesten oder relativ wenig abriebfesten festen Substanzen dispergiert ist;
f) Trockenen des dritten Harzes.

2. Verfahren nach Anspruch 1, **dadurch gekennzeichnet, dass** vor dem Auftragen der Mischung das im Wesentlichen trockene bahnenförmige Material einen Nassrückstand an flüchtigen Substanzen (bestimmt in einem Ofen bei 160 °C für 5 Minuten) von weniger als ungefähr 14 Gew.-% hat.

3. Verfahren nach Anspruch 1 oder 2, **dadurch gekennzeichnet, dass** das bahnenförmige Material ein nichtimprägniertes Papiermaterial ist.

4. Verfahren nach Anspruch 1 oder 2, **dadurch gekennzeichnet, dass** das bahnenförmige Material ein vorimprägniertes, sogenanntes bahnenförmiges "prepreg" Material ist; wobei in diesem Fall das Verfahren die Schritte umfasst: i) Imprägnieren des bahnenförmigen Material mit einem zweiten Duroplastharz; ii) Trocknen des vorimprägnierten bahnenförmigen Materials um das zweite Duroplastharz durch Vernetzen zu polymerisieren; und iii) gleichmäßiges Auftragen und Verteilen der Mischung auf wenigstens einer Oberfläche des getrockneten vorimprägnierten bahnenförmigen Materials.

5. Verfahren nach Anspruch 4, **dadurch gekennzeichnet, dass** nach dem Trocknen und vor dem Auftragen der Mischung das getrocknete vorimprägnierte bahnenförmige Material einen Nassrückstand an flüchtigen Substanzen (bestimmt in einem Ofen bei 160 °C für 5 Minuten) von 7 bis 14 Gew.-% hat.

6. Verfahren nach einem der vorherigen Ansprüche, **dadurch gekennzeichnet, dass** das erste Duroplastharz während der Schritte des Erzeugens und Auftragens der Mischung kontinuierlich gemischt wird und in bevorzugt turbulenter Bewegung gehalten wird.

7. Verfahren nach einem der vorherigen Ansprüche, **dadurch gekennzeichnet, dass** der Schritt des Auftragens der Mischung von einer Auftragvorrichtung durchgeführt wird, umfassend eine Spenderquelle und wenigstens eine Auftragswalze, die so angeordnet ist, dass sie im Wesentlichen die erste Oberfläche des bahnenförmigen Materials entlang einer generierenden Berührungslinie kontaktiert, um die Mischung von der Spenderquelle auf die erste Oberfläche zu transferieren; während auf einer zweiten Oberfläche des bahnenförmigen Materials, die sich gegenüber der ersten Oberfläche befindet, und an der generierenden Berührungslinie kein Träger für das bahnenförmige Material bereitgestellt wird.

8. Verfahren nach dem vorherigen Anspruch, **dadurch gekennzeichnet, dass** es weiterhin einen Schritt des Rückführens der Mischung umfasst, worin die Mischung, die von der Spenderquelle abgegeben und nicht auf die erste Oberfläche des bahnenförmigen Materials aufgetragen wird, wiedergewonnen und in die Spenderquelle rückgeführt wird.

9. Verfahren nach einem der vorherigen Ansprüche, **dadurch gekennzeichnet, dass** während dem Schritt des Erzeugens der Mischung, wenigstens ein Zusatzstoff zur Viskositätskontorolle zur Mischung hinzugefügt wird, der ausgewählt ist aus der Gruppe umfassend filmbildende Mittel und der bevorzugt zu thermischem dreidimensionalem Vernetzen in der Lage ist.

10. Verfahren nach einem der vorherigen Ansprüche, **dadurch gekennzeichnet, dass** die Duroplastharze wasserbasierte Harze sind, die beispielsweise ausgewählt sind aus der Gruppe umfassend Melamin-, Phenol- Harnstoffharze und Mischungen davon; wobei die pulverförmige abriebfeste Substanz Aluminiumoxid (Al₂O₃, Korund) ist.

11. Verfahren nach einem der vorherigen Ansprüche, **dadurch gekennzeichnet, dass** die Schritte des Auftragens der Mischung und Trocknen des bahnenförmigen Materials, das mit der Mischung beschichtet ist, ein oder mehrere Male wiederholt werden, um übereinanderliegenden Schichten zu bilden.

## Revendications

1. Procédé de production de revêtements de protection hautement résistants à l'abrasion, en particulier pour sols et surfaces de travail, comprenant les étapes consistant à :
a) préparer un mélange d'une substance en poudre résistante à l'abrasion dispersée de façon homogène dans une première résine polymère thermodurcissable ;
b) utiliser un matériau en feuille sensiblement sec contenu un résidu faiblement humide de substances volatiles ;
c) appliquer et répartir ledit mélange de façon homogène sur au moins une surface dudit matériau en feuille sensiblement sec ;
d) sécher ledit matériau en feuille recouvert dudit mélange pour former un revêtement renfermant ladite substance en poudre résistante à l'abrasion ;
le procédé étant **caractérisé en ce qu'**il comprend également, après ladite étape d'application dudit mélange et ladite étape de séchage dudit matériau en feuille recouvert dudit mélange, les étapes consistant à :
e) appliquer sur ledit revêtement renfermant ladite substance en poudre résistante à l'abrasion au moins une couche d'une troisième résine polymère thermodurcissable contenant un agent de remplissage particulaire dans lequel sont dispersées des substances solides non abrasives ou relativement non abrasives ; et
f) sécher ladite troisième résine.

2. Procédé selon la revendication 1, **caractérisé en ce que**, avant l'application dudit mélange, ledit matériau en feuille sensiblement sec comporte un résidu humide de substances volatiles (déterminé dans un four à 160° pendant 5 minutes) de moins d'approximativement 14 % en poids.

3. Procédé selon la revendication 1 ou 2, **caractérisé en ce que** ledit matériau en feuille est un matériau en papier non imprégné.

4. Procédé selon la revendication 1 ou 2, **caractérisé en ce que** ledit matériau en feuille est un matériau en feuille préimprégné ; auquel cas, le procédé comprend les étapes consistant à : i) imprégner ledit matériau en feuille d'une deuxième résine polymère thermodurcissable ; ii) sécher ledit matériau en feuille préimprégné pour polymériser-réticuler ladite deuxième résine polymère thermodurcissable ; et, iii) appliquer et répartir ledit mélange de façon homogène sur au moins une surface dudit matériau en feuille préimprégné séché.

5. Procédé selon la revendication 4, **caractérisé en ce que**, après le séchage et avant l'application dudit mélange, ledit matériau en feuille préimprégné séché comporte un résidu humide de substances volatiles (déterminé dans un four à 160° pendant 5 minutes) de 7 à 14 % en poids.

6. Procédé selon l'une des revendications précitées, **caractérisé en ce que** ladite première résine polymère thermodurcissable est agitée en continu et maintenue dans un mouvement de préférence turbulent pendant lesdites étapes de préparation et d'application dudit mélange.

7. Procédé selon l'une des revendications précitées, **caractérisé en ce que** ladite étape d'application dudit mélange est effectuée par un dispositif de distribution comprenant une fontaine, et au moins un rouleau-applicateur positionné sensiblement en contact avec ladite première surface du matériau en feuille le long d'une ligne de contact génératrice pour transférer ledit mélange de ladite fontaine vers ladite première surface ; alors que, sur une seconde surface, opposée à ladite première surface, du matériau en feuille et au niveau de ladite ligne de contact génératrice, aucun support pour ledit matériau en feuille n'est prévu.

8. Procédé selon la revendication précitée, **caractérisé en ce qu'**il comprend également une étape consistant à remettre en circulation ledit mélange, et dans lequel ledit mélange distribué par ladite fontaine et non déposé sur ladite première surface du matériau en feuille est récupéré et renvoyé à ladite fontaine.

9. Procédé selon l'une des revendications précitées, **caractérisé en ce que**, au cours de ladite étape de préparation dudit mélange, au moins un additif de régulation de viscosité, choisi dans le groupe comprenant des filmogènes et pouvant de préférence effectuer une réticulation tridimensionnelle thermique, est ajouté audit mélange.

10. Procédé selon l'une des revendications précitées, **caractérisé en ce que** lesdites résines polymères thermodurcissables sont des résines à base d'eau choisies, par exemple, dans le groupe comprenant des résines mélamines, des résines phénoliques, des résines d'urée et des mélanges de celles-ci ; ladite substance en poudre résistante à l'abrasion étant de l'oxyde d'aluminium (Al₂O₃, corindon) .

11. Procédé selon l'une des revendications précitées, **caractérisé en ce que** lesdites étapes d'application dudit mélange et de séchage dudit matériau en feuille recouvert dudit mélange sont répétées une ou plusieurs fois pour former des couches de revêtement superposées respectives.
